# EUROPEAN PATENT SPECIFICATION

(11) **EP 0 178 502 B1**
(45) Date of publication and mention of the grant of the patent: **13.09.1989**
(21) Application number: 85112130.1
(22) Date of filing: 24.09.1985
(51) Int. Cl.: C22C 1/02

(54) **Alloying process**
Verfahren zur Herstellung von Legierungen
Procédé pour la fabrication d'alliages

(30) Priority: 27.09.1984 US 654736; 27.09.1984 US 654735
(43) Date of publication of application: 23.04.1986
(73) Proprietor: ALUMINUM COMPANY OF AMERICA, Pittsburgh, PA 15219 (US)
(72) Inventor: Eckert, Charles E., Pittsburgh Pennsylvania (US); Miller, Ronald E., Murrysville Pennsylvania (US)
(74) Representative: Baillie, Iain Cameron

(56) References cited:
- FR-A- 2 211 533
- US-A- 3 947 265

## Description

The invention relates generally to a method for adding alloying elements to molten metals. More particularly, however, it relates to the addition of elements which normally dissolve slowly and with difficulty in molten metals, particularly aluminum.

Many different methods have been employed to add alloying elements to molten metals. Conventional methods typically add the elements directly to the melt in theform of a lump, a bar orthe like. In some cases, they are added directly to molten metal being tapped into a ladle, and in other cases, they may be placed in the ladle prior to tapping.

Another method for adding alloying elementsto molten metals, particularly molten steel, is disclosed in U.S. Patent 3,768,999 ro Ohkubo et al. In Ohkubo, alloying is accomplished by feeding a wire rod into the molten metal. The rod is coated with additives for the molten metal and an organic binder which decomposes into gaseous products in the molten metal. The generated gas stirs the molten metal and thus uniformly incorporates the added components throughout the molten metal.

U.S. Patent 3,729,309 to Kawawa also discloses a method for adding alloying elements in the form of a wire rod to molten metals. The rod has a controlled size and is added to a molten metal bath by inserting it at a controlled speed, so as to produce a refined and purified metal alloy.

The above methods of adding alloying elements to molten metal work fairly well with alloying elements which dissolve and disperse easily in the molten metal. However, such methods do not work so well with elements having limited liquid solubility such as Pb, Bi and Sn and high oxidizing potential such as Mg and Zn.

U.S. Patent 3,947,265 to Guzowski et al proposes a solution to the problem of adding such "hard-to- alloy" materials to molten metal. The process employs a high current arc which is formed between the molten base metal and the alloying addition. The alloying addition is passed through the arc where it is melted and converted into a spray of finely divided superheated molten particles. In such a condition, the particles are able to rapidly dissolve in the molten metal upon contact therewith. While the Guzowski concept of alloying is certainly an interesting one, a need still exists for a process capable of providing improved results.

In accordance with the present invention, there is provided a process for adding material to a molten metal media comprising the steps of:
(a) providing a body of molten media;
(b) providing a chamber means having an open discharge end positioned within said media body;
(c) supplying said chamber means with a gas comprising an ionizable gas under sufficient pressure to maintain an interior molten media surface substantially at said chamber's discharge end region;
(d) supplying said material to a site within said chamber above said interior molten media surface;
(e) conducting an electric arc between said material at said site and said interior molten media surface and maintaining a plasm substantially extending from said site within said chamber to said interior molten media surface; and
(f) maintaining said plasma at a sufficient energy to convert said material into a superheated spray substantially within said plasma projected toward said interior molten media surface;
(g) said supplying of said gas to said chamber being of sufficient rate to project said material into said media so as to enhance entry of said material into said media.

In an embodiment of the invention, the chamber means is elongate and has an upper inlet, at least a portion of which is located above the upper surface of the molten media, the material being fed into the chamber through said inlet, and the interior surface of the body of molten media being maintained at a depth below said exterior surface such that at least 50% of material being added to the molten media is recovered in the molten media.

In accordance with the present invention, a method is provided for adding alloying material to a molten metal media, such as molten aluminum. The method includes the step of converting the alloying material into a spray of superheated alloy material and directing the spray into the molten metal media at a predetermined depth below the media's surface, the depth having been determined beforehand to enhance dissolution and dispersion of the alloying material into the molten media.

In a preferred embodiment, the alloying material is converted into the spray of superheated alloy material in a spark cup means which is at least partially immersed in the molten media body. The spark cup has a lower open end which is exposed to the molten media and an upper inlet, at least a portion of which is located above the exposed or exterior surface of the molten media. The lower open end of the spark cup is maintained or immersed a predetermined depth below the surface of the molten media. The alloying material, preferably in the form of an elongated element having a free end, is continually fed into the spark cup through its upper inlet, and an electrical arc discharge between the submerged molten metal surface and the alloying element in the spark cup is maintained with a current that exceeds the globular/spray transition current density of the alloying material. At such a cu rrent, the free or exposed end of the alloying element is converted into a spray of superheated material. Arc shielding gas is continually supplied to the spark cup through its upper inlet also. In addition to shielding the arc discharge, the gas slightly pressurizes the spark cup and thereby prevents molten media from entering its open end. As such, a submerged interior surface of molten metal media is created in the spark cup's open end at the aforementioned predetermined depth. The shielding gas also carries or projects the superheated spray of alloy material into the molten media through the submerged molten metal surface so as to permit dissolution and dispersion of the alloy material in the media. The predetermined depth of immersion has been found to significantly enhance dispersion and dissolution of the alloying material into the media.

The present invention also provides a lead alloyed, aluminum based article having high machinability. The article is produced by converting lead alloy material into a spray of superheated alloy material which is injected into a bath of molten aluminum at a predetermined depth below the molten bath's surface. The spray is formed by establishing an electrical arc discharge between a submerged surface of the molten media and the alloying material. The discharge is maintained with a current that exceeds the globular/spray transition current density of the alloying material. The spray of superheated alloying material is directed onto the submerged interior surface of the media where dissolution and dispersion of the alloy material into the media take place. The submerged surface is maintained at the predetermined depth below the bath's surface having been found to enhance said dissolution and dispersion of the lead into molten aluminum bath. The article so produced has acicular shaped particles of lead which are smaller and more uniformly sized and dispersed than those which are made by adding lead at the surface of the molten aluminum or at a depth above the aforesaid predetermined depth.
Figure 1 illustrates an embodiment of the present invention.
Figure 2 illustrates the spark cup depicted in Figure 1.
Figure 3 is a graph plotting alloy dissolution rate in pounds per minute versus spark cup immersion depth.
Figure 4 is a graph illustrating the relationship of actual recovery in percentages versus immersion depth in inches.

Figure 1 illustrates the addition of a wire 10 of alloying material into a bath or melt 12 of molten media in a flow-through furnace 14. The surface of melt 12 is referred to herein as exposed or exterior surface 16. Wire 10 is being fed by a feeder 18 which passes it through a triplex feed cable 20 into a spark cup 22, the spark cup being partially immersed in melt 12. In spark cup 22, alloy wire 10 is converted into a spray 24 of superheated alloy material by passing it through a plasma arc discharge (not numbered). The plasma arc discharge is established between a submerged surface 26 of the molten metal which is maintained within an open end 28 of spark cup 22 and a free end 30 of alloy wire 10. The arc discharge is shielded with a shielding gas 32, preferably argon, which is provided via feed cable 20 by an arc shielding gas source 34. In addition to providing a shielding atmosphere for the arc in the spark cup, the shielding gas source 34 pressurizes the spark cup at a pressure which is sufficient to prevent molten metal from entering open end 28 of the spark cup. Such pressurization also facilitates maintenance of the aforementioned submerged surface at a certain predetermined depth below exposed surface 16 (more on this, infra). Returning to Figure 1, it will be seen that the arc discharge is powered by a constant current power supply source 36 (more on this, infra). Melt 12 serves as an anode with wire 10 serving as a consumable electrode. The electrical circuit leading back to current source 36 is completed by a return wire 38 which is attached to a rod 40 immersed in melt 12. The superheated spray produced by the arc discharge is directed or projected by the supply of shielding gas onto submerged surface 26 where the alloy material rapidly dissolves and disperses in melt 12. The gas is preferably supplied at a flow rate that maximizes the projection of the spray into the melt. An impeller 42 or agitating means is also provided to further enhance dispersion of the alloy material throughout the melt. Spray 24 can be maintaiined as long as is desired by continually advancing or feeding the alloying wire into the spark cup. Feeder 18 can also be controlled to maintain or vary the rate at which wire 10 is fed into the spark cup.

The alloying material can be provided in wire form, as described above, or in the form of rod, tube, strip or in powdered form wherein the powders are encased in a hollow tube made from a suitable metal which has been swaged or otherwise worked to reduce its diameter and compact the powdered material in the tube. The only real limitation on the form of the alloying is that it should have a form which permits it to be fed into the feed cable in a seal-tight fashion, thereby enabling the pressurized atmosphere in the spark cup to be maintained. If the pressurized atmosphere in the spark cup is not maintained, molten metal will, quite obviously, enter the spark cup through its open end 28, thereby raising submerged surface 26 to a depth above its predetermined depth. Such raising of submerged surface 26 will result in lower dissolution and dispersion rates. (The importance of maintaining submerged surface 26 at its predetermined depth will be discussed in more detail, infra.) While no means for sealing the wire is depicted in Figure 1, those skilled in the art will be aware of numerous means having the capability of providing an effective seal. Such means could include elastomer and pneumatic seals. In addition, feeder 18 is preferably a consistent feed rate tractor drive.

Constant current source 36 is preferably of the type which maintains a relatively constant current regardless of voltage fluctuations. The arc produced thereby has self-stabilizing characteristics and is relatively insensitive to changes in arc length which might be caused by fluctuations in the submerged molten metal depth. It may also be desirable in certain situations to further enhance arc stability by seeding the plasma discharge with certain additives, such as alkali metals which are known to promote arc stability. Arc stability can also be enhanced by using various fluxes known to those skilled in the relevant art.

As mentioned in U.S. Patent 3,947,265 to Guzowski, it may be desirable to add a high frequency, high voltage component to the arc which is particularly useful if AC current is used. This apparently reduces the tendency of the arc to extinguish every time the voltage passes through zero, increases the stability of the arc and makes initiation of the arc less difficult.

An important aspect of the present invention requires that the current supplied by power source 36 exceed the globular/spray transition current density of the alloyed material. As used herein, the globular/spray transition current density defines the boundary line separating the two different types of metal transfer that are capable of occurring in the plasma arc discharge. (As pointed out by Guzowski in U.S. Patent 3,947,265, this transition point can vary with such factors as alloy type, wire size and wire speed.) In cases with current densities below the transition point, alloy material being transferred through the arc detached into large drops which dissolve and disperse slowly in the molten metal media. At current densities above the transition point, the transfer mechanism changes causing the alloy material to convert a fine spray of superheated alloy material. In this condition, the alloy material rapidly dissolves and disperses in the molten media upon contact with submerged surface 26.

Shielding gas 32 carrying or projecting spray 24 into the melt also typically enters the melt. This, however, should not introduce or cause any melt contamination since such gas simply escapes from the melt by bubbling through the melt to exterior surface 16. As previously mentioned, the preferred shielding gas is argon; however, other shielding gases, such as helium, carbon monoxide and carbon dioxide, may also be used in appropriate situations.

The spark cup is preferably cylindrically shaped. Such a shape provides a relatively high spark cup surface area to volume ratio which facilitates conductive heat transfer from the spark cup to the melt. It is important to facilitate such heat transfer to prevent the spark cup from overheating. Moreover, those skilled in the relevant art will appreciate that such heat transfer to the melt is advantageous in that it provides a convenient way of adding heat to the melt, thereby reducing furnace fuel needs. Conventional alloy adding processes such as that disclosed in Guzowski et al U.S. Patent No. 3,947,265 do not add much, if any, heat to their respective melts. For example, most of the heat generated during melting of the alloy material in Guzowski et al is lost to the atmosphere since the superheated spray is formed entirely above the melt surface.

The spark cup's cylindrical shape also enhances projection of the shielding gas carrying the superheated spray into the melt. Such projection is important in that it enhances dissolution and dispersion of the alloying material into the melt. While a cylindrical shape is preferred, other shapes, such as an inverted frustoconical shape, which provide enhanced projection and heat transfer are considered to be within the purview of the present invention.

The spark cup's composition is another important aspect of the present invention. Preferably, it is made from material having the following characteristics:
1. High radiation heat transfer so as to maximize the transfer of radiation heat from the arc discharge to the melt, thereby reducing the possibility of overheating in the spark cup.
2. High resistance to thermal and mechanical shock.
3. High thermal and chemical stability in the melt. Borosilicate, alumina, mullite and silica are some materials known to possess the desired characteristics.

Another briefly alluded to but important aspect of the present invention is directed to immersing the spark cup and maintaining submerged surface 26 in the open end of the spark cup at its predetermined depth below exposed surface 16. Such depth will be referred to hereinafter as the predetermined immersion depth. It has been found that a difference of one or two inches in the immersion depth can have a significant impact upon the rate at which alloying material dissolves and disperses in the molten media. Figures 3 and 4 set forth test data from experiments conducted to determine the effects of immersion depth upon dissolution and dispersion. Figure 3 sets forth data respecting dissolution rate versus immersion depth, and Figure 4 shows actual recovery in percentages versus immersion depth. The goal of the experiments was to add 0.5% lead to a substantially lead-free body of molten aluminum. The experiments were conducted with a setup similar to that disclosed in Figure 1 except that a constant voltage supply source was used instead of the preferred constant current supply source. The flow-through furnace used in the experiments contained approximately 454 Kgs (1000 pounds) of aluminum. The bath of molten aluminum in the furnace had a depth of approximately 76 cm (30 inches) with a diameter of approximately 58 cm (23 inches). Lead wire of 3.175 mm (8 inch) diameter was fed into a borosilicate spark cup at a feed rate of about 76 cm (30 inches) per minute via a triplex feed cable. The spark cup was cylindrically shaped and had a lower opening similar to that described in Figure 1 with a diameter of approximately five centimeters. The spark cup's length to diameter ratio was approximately 6 to 1. Argon shielding gas was fed into the spark cup via the feed cable at a flow rate of about 0.28 standard m³/hr (10 standard ft³/hr). A plasma arc discharge was established in the spark cup between the free end of the lead wire and the submerged molten metal surface at a voltage of about 35 volts and a current of about 125 amperes, which translates into a current density of about 1550 amps/cm² (10,000 amp/ in²). As such, the free end of the wire melted and converted into an axial spray of superheated alloy material upon entering the arc discharge. The spray was directed onto the submerged melt surface by the shielding gas. After adding an appropriate amount of lead wire to the bath of molten aluminum, the alloyed molten aluminum was continuously cast into several ingots having dimensions of 15 cm x 15 cm x 91 cm (6 in. x 6 in. x 36 in.).

From Figure 3, those skilled in the art will appreciate that a dramatic increase in lead's dissolution rate (that is, the rate at which lead dissolved into the molten media) resulted when the spark cup immersion depth was increased from 12.7 to 15 cm (5 to 6 inches). It will be noted that further increases in immersion depth did not seem to have much of an effect upon the dissolution rate. Similarly, in Figure 4, it can be seen that actual recovery in percentages increased dramatically when the immersion depth was increased from 10 to 15 cm (4 to 6 inches). Moreover, further increases in the immersion depth showed further increases in actual recovery; however, not nearly as dramatic as those that occurred from 10 to 15 cm (4 to 6 inches). Actual recovery was measured by optical emission spectroscopy. Metallographic examination revealed that the particles of lead in the cast ingot were smaller, more acicular shaped and more uniformly sized and dispersed than those added by conventional methods. Moreover, it is believed that such ingot provided by the present invention has improved machinability.

While the immersion depth providing enhanced dissolution and dispersion in accordance with the present invention will vary with the material being added, bath size, bath flow rate, alloy feed rate and size, inter alia, and will have to be determined for each setup, those skilled in the relevant art will appreciate that the method and apparatus of the present invention can result in greatly increased dissolution rates, particularly for alloy material with limited solubility, such as lead, bismuth and tin and for high oxidizable materials such as magnesium and zinc.

Those skilled in the art will also appreciate that the present invention is amenable to continuous casting processes. Continuous casting processes are those that permit the continual flow of metal from a melting furnace into a casting mold. Since continuous casting usually proceeds at a uniform rate, it will be easy to calculate the desired alloy feed rate with the method of the present invention. The invention, however, is particularly amenable to continuous casting processes wherein the casting rate varies. Suitable instrumentation can be installed on the casting line to detect any changes in the casting rate which can then be used to make adjustments in the alloy feed rate.

## Claims

1. A process for adding material to a molten metal media comprising the steps of:
(a) providing a body of molten media;
(b) providing a chamber means having an open discharge end positioned within said media body;
(c) supplying said chamber means with a gas comprising an ionizable gas under sufficient pressure to maintain an interior molten media surface substantially at said chamber's discharge end region;
(d) supplying said material to a site within said chamber above said interior molten media surface;
(e) conducting an electric arc between said material at said site and said interior molten media surface and maintaining a plasma substantially extending from said site within said chamber to said interior molten media surface; and
(f) maintaining said plasma at a sufficient energy to convert said material into a superheated spray substantially within said plasma projected toward said interior molten media surface;
(g) said supplying of said gas to said chamber being of sufficient rate to project said material into said media so as to enhance entry of said material into said media.

2. A process according to claim 1, in which the chamber means is elongate and has an upper inlet, at least a portion of which is located above the upper surface of the molten media, the material being fed into the chamber through said inlet, and the interior surface of the body of molten media being maintained at a depth below said exterior surface such that at least 50% of material being added to the molten media is recovered in the molten media.

3. A process according to claim 1 or 2, wherein said interior molten media surface is maintained at a predetermined depth below the upper surface of the molten media, said depth being sufficient to enhance dissolution and dispersion of the material into said media.

4. A process according to any one of the preceding claims, wherein substantial heat is transmitted to the molten media through the chamber portion submerged in the media.

5. A process according to any one of the preceding claims in which the molten media comprises aluminum.

6. A process according to any one of the preceding claims in which the added material is supplied to the chamber means in the form of solid wire or rod.

7. A process according to any one of the preceding claims in which the gas comprises a nonreactive gas.

8. A process according to claim 7 in which the gas is seeded with at least one additive to promote arc stability or oxygen scavenging.

9. A process according to any one of the preceding claims, in which the electric arc is formed by a direct current.

10. A process according to any one of the preceding claims, in which the length of the chamber along the direction of projection into the molten media exceeds the transverse dimension of the chamber outlet.

11. A process according to any one of the preceding claims in which material added comprises one or more of lead, bismuth, antimony, magnesium, zinc or copper.

12. A process according to any one of the preceding claims, in which the chamber means is made from alumina, borosilicate, mullite or silica.

13. A process according to any one of the preceding claims, in which the molten media is agitated to further enhance dispersion of the material within said media.

## Patentansprüche

1. Verfahren zum Versetzen einer Metallschmelze mit einen Gut, mit folgenden Schritten:
(a) es wird ein aus einer Schmelze bestehender Körper gebildet;
(b) es wird eine Kammeranordnung geschaffen, die ein in der Schmelze offenes Austrittsende hat;
(c) die Kammeranordnung wird mit einem Gas beschickt, das mindestens teilweise aus einem ionisierbaren Gas unter einem so hohen Durch besteht, daß im wesentlichen in dem Austrittsendbereich der Kammer eine innere Schmelzefläche aufrechterhalten wird;
(d) das genannte Gut wird einer in der Kammer oberhalb der inneren Schmelzefläche gelegenen Stelle zugeführt;
(e) zwischen dem an der genannten Stelle befindlichen Gut und der inneren Schmelzefläche wird ein Lichtbogen gezogen, und in der Kammer wird ein Plasma aufrechterhalten, das sich im wesentlichen von der genannten Stelle bis zu der inneren Schmelzefläche erstreckt; und
(f) des genannte Plasma wird mit einem so hohen Energiegehalt aufrechterhalten, daß das genannte Gut in einen überhitzten Sprühnebel umgewandelt wird, der im wesentlichen in dem Plasma zu der inneren Schmelzefläche vorgetrieben wird;
(g) die Kammer wird mit dem Gas in einer solchen Menge beschickt, daß durch den Vortrieb des genannten Gutes in der Schmelze der Eintritt des genannten Gutes in die Schmelze unterstützt wird.

2. Verfahren nach Anspruch 1, dadurch gekennzeichnet, daß die Kammeranordnung langgestreckt ist und einen oberen Eintritt besitzt, der sich mindestens zum Teil oberhalb der oberen Fläche der Schmelze befindet und durch den hindurch das Gut in die Kammer eingeleitet wird, und daß die innere Fläche des aus der Schmelze bestehenden Körpers in einer solchen Tiefe unterhalb der genannten oberen Fläche gehalten wird, daß mindestens 50% des der Schmelze zugesetzten Gutes in dieser gewonnen wird.

3. Verfahren nach Anspruch 1 oder 2, dadurch gekennzeichnet, daß die innere Schmelzefläche in einer solchen vorherbestimmten Tiefe unter der oberen Schmelzefläche gehalten wird, daß das Auflösen und Dispergieren des Gutes in der Schmelze unterstützt wird.

4. Verfahren nach einem der vorhergehenden Ansprüche, dadurch gekennzeichnet, daß über den in der Schmelze untergetauchten Kammerteil der Schmelze eine beträchtliche Wärmemenge zugeführt wird.

5. Verfahren nach einem der vorhergehenden Ansprüche, dadurch gekennzeichnet, daß die Schmelze mindestens teilweise aus Aluminium besteht.

6. Verfahren nach einem der vorhergehenden Ansprüche, dadurch gekennzeichnet, daß das zuzusetzende Gut der Kammeranordnung in Form von massivem Draht- oder Stabmaterial zugeführt wird.

7. Verfahren nach einem der vorhergehenden Ansprüche, dadurch gekennzeichnet, daß das Gas mindestens teilweise aus einem reaktionsunfähigen Gas besteht.

8. Verfahren nach Anspruch 7, dadurch gekennzeichnet, daß das Gas mit mindestens einem Zusatzstoff geimpft wird, um den Lichtbogen zu stabilisieren oder Sauerstoff zu entfernen.

9. Verfahren nach einem der vorhergehenden Ansprüche, dadurch gekennzeichnet, daß der Lichtbogen mit Gleichstrom erzeugt wird.

10. Verfahren nach einem der vorhergehenden Ansprüche, dadurch gekennzeichnet, daß die Länge der Kammer in der Richtung des Vortriebes in die Schmelze größer ist als die Querabmessung am Austritt der Kammer.

11. Verfahren nach einem der vorhergehenden Ansprüche, dadurch gekennzeichnet, daß das hinzuzufügende Gut mindestens teilweise aus einer oder mehreren der nachstehenden Substanzen besteht: Blei, Wismut, Antimon, Magnesium, Zink oder Kupfer.

12. Verfahren nach einem der vorhergehenden Ansprüche, dadurch gekennzeichnet, daß die Kammeranordnung aus Aluminiumoxid, Borsilikat, Mullit oder Siliciumdioxid besteht.

13. Verfahren nach einem der vorhergehenden Ansprüche, dadurch gekennzeichnet, daß zum weiteren Unterstützen des Dispergierens des Gutes in der Schmelze diese bewegt wird.

## Revendications

1. Procédé d'addition d'un matériau dans un milieu métallique en fusion, dans lequel:
(a) on prépare une masse de milieu en fusion;
(b) on met en place une chambre comportant une extrémité d'évacuation ouverte, disposée dans cette masse de milieu;
(c) on introduit, dans la chambre, un gaz comprenant un gaz ionisable, sous une pression suffisante pour maintenir une surface intérieure du milieu en fusion, à peu près au niveau de la partie d'extrémité d'évacuation de la chambre;
(d) on introduit le matériau dans la chambre, au niveau d'une zone située au-dessus de la surface intérieure du milieu en fusion;
(e) on établit un arc électrique entre le matériau au niveau de ladite zone et de la surface intérieure du milieu en fusion, et on maintient un plasma s'étendant à peu près à partir de ladite zone dans la chambre jusqu'à la surface intérieure du milieu en fusion; et
(f) on maintient le plasma à une énergie suffisante pour convertir le matériau en un jet pulvérisé surchauffé, s'étendant à peu près dans le plasma en direction de la surface intérieure du milieu en fusion;
(g) l'introduction du gaz dans la chambre, étant effectuée à une vitesse suffisante pour projeter le matériau dans le milieu en fusion de façon à favoriser la pénétration du matériau dans ce milieu.

2. Procédé selon la revendication 1, dans lequel la chambre est allongée et comporte un orifice d'entrée supérieur, au moins une partie de celle-ci étant située au-dessus de la surface supérieure du milieu en fusion, le matériau étant introduit dans la chambre, à travers l'orifice d'entrée, et la surface intérieure de la masse de milieu en fusion étant maintenue à une profondeur située en-dessous de la surface extérieure, de telle façon qu'au moins 50% du matériau additionné dans le milieu en fusion, soient récupérés dans le milieu en fusion.

3. Procédé selon la revendication 1 ou 2, dans lequel la surface intérieure du milieu en fusion, est maintenue à une profondeur prédéterminée sous la surface supérieure du milieu en fusion, cette profondeur étant suffisante pour favoriser la dissolution et la dispersion du matériau dans ce milieu.

4. Procédé selon l'une quelconque des revendications précédentes, dans lequel une quantité importante de chaleur est transmise au milieu en fusion, à travers la partie de la chambre, immergée dans le milieu.

5. Procédé selon l'une quelconque des revendications précédentes, dans lequel le milieu en fusion, comprend de l'aluminium.

6. Procédé selon l'une quelconque des revendications précédentes, dans lequel le matériau additionné, est introduit dans la chambre sous la forme d'un fil ou d'une tige plein.

7. Procédé selon l'une quelconque des revendications précédentes, dans lequel le gaz comprend un gaz non réactif.

8. Procédé selon la revendication 7, dans lequel on disperse dans le gaz au moins un additif destiné à favoriser la stabilité de l'arc ou l'absorption de l'oxygène.

9. Procédé selon l'une quelconque des revendications précédentes, dans lequel l'arc électrique est formé à partir d'un courant continu.

10. Procédé selon l'une quelconque des revendications précédentes, dans lequel la longueur de la chambre, le long de la direction de projection dans le milieu en fusion, est supérieure à la dimension transversale de l'orifice de sortie de la chambre.

11. Procédé selon l'une quelconque des revendications précédentes, dans lequel le matériau additionné, comprend un ou plusieurs éléments choisis parmi le plomb, le bismuth, l'antimoine, le magnésium, le zinc et le cuivre.

12. Procédé selon l'une quelconque des revendications précédentes, dans lequel la chambre est réalisée en alumine, en borosilicate, en mullite ou en silice.

13. Procédé selon l'une quelconque des revendications précédentes, dans lequel le milieu en fusion est agité pour favoriser encore la dispersion du matériau dans le milieu.
